



US005942464A

# United States Patent [19]

Vaughn et al.

[11] Patent Number: 5,942,464

[45] Date of Patent: Aug. 24, 1999

[54] **METHOD AND APPARATUS FOR PRINTING**[75] Inventors: **Larry Vaughn**, Indiana, Pa.; **John G. Whitaker**, Chattanooga, Tenn.[73] Assignee: **Larry F. Vaughn**, Indiana, Pa.[21] Appl. No.: **09/005,744**[22] Filed: **Jan. 12, 1998****Related U.S. Application Data**

[60] Continuation-in-part of application No. 08/744,243, Nov. 5, 1996, Pat. No. 5,707,924, which is a division of application No. 08/551,824, Nov. 7, 1995, Pat. No. 5,830,823.

[51] **Int. Cl.<sup>6</sup>** ..... **B41M 5/165**[52] **U.S. Cl.** ..... **503/200**; 427/150; 427/180; 427/372.2; 428/304.4; 428/321.5; 503/215; 503/216[58] **Field of Search** ..... 427/150-152, 427/180, 372.2; 428/304.4, 321.5; 503/200, 215, 216[56] **References Cited****U.S. PATENT DOCUMENTS**

3,578,482 5/1971 Whitaker et al. ..... 117/38

|           |         |                      |          |
|-----------|---------|----------------------|----------|
| 3,819,396 | 6/1974  | Vincent et al. ....  | 117/36.2 |
| 4,232,083 | 11/1980 | Buerkley et al. .... | 428/307  |
| 4,262,936 | 4/1981  | Miyamoto ....        | 503/212  |
| 4,302,393 | 11/1981 | Garner et al. ....   | 260/335  |
| 4,379,178 | 4/1983  | Meadows et al. ....  | 427/1    |
| 4,699,077 | 10/1987 | Meadows et al. ....  | 118/31.5 |
| 5,009,919 | 4/1991  | Vassiliades ....     | 427/1    |
| 5,454,600 | 10/1995 | Floyd ....           | 293/78   |

*Primary Examiner*—Bruce H. Hess*Attorney, Agent, or Firm*—Luedeka, Neely & Graham PC

[57]

**ABSTRACT**

The invention described herein relates to methods and systems for printing. More specifically, the present invention provides methods and systems for printing using a disposable substrate containing an essentially dry layer of micro-capsules which contain a colorless dye compound or dye developing compound and a substantially dry layer of containing a complementary compound in a second substrate region for reaction with the dye or dye developing compound to form a visible image. The disposable printing system according to the invention provides a reduced availability for bacterial growth and transfer due to its essentially dry characteristics.

**20 Claims, 4 Drawing Sheets**



***Fig. 1***



***Fig. 2***



Fig. 3



Fig. 4



**Fig. 5**



**Fig. 6**



Fig. 7

## METHOD AND APPARATUS FOR PRINTING

This application is a continuation-in-part of application Ser. No. 08/744,243, filed Nov. 5, 1996, now U.S. Pat. No. 5,707,924, which is a division of application Ser. No. 08/551,824, filed Nov. 7, 1995, now U.S. Pat. No. 5,830,823.

## SUMMARY OF THE INVENTION

The present invention relates to essentially dry colorless dyes and developers and to methods for making an essentially dry printing system using colorless dyes and developers therefor.

According to one aspect, the invention provides an essentially dry ink pad containing an essentially colorless composition for use with a complementary essentially colorless compound to develop a visible image. The ink pad comprises a porous substrate impregnated with a substantially dry layer of microcapsules, said microcapsules containing an essentially colorless dye compound, oleaginous carrier fluid and a fragrance.

According to another aspect, the invention provides a method for making an essentially dry printing system. The method comprises milling an aqueous gelatin mixture containing water, a solution containing from about 10 to about 20 percent by weight of an electron donating dye compound and from about 80 to about 90 percent by weight of an oleaginous material to a particle size of about 40 to about 80 microns, dispersing the milled aqueous gelatin mixture in an aqueous gum arabic solution while mixing the dispersion at a speed sufficient to maintain the particle size, cooling the dispersed mixture to a temperature in the range of from about 5 to about 15° C., adding a cross-linking agent to the cooled mixture to form microcapsules, maintaining the cooled mixture under agitation for from about 10 to about 20 hours at a pH of about 4.5, removing water from the mixture containing microcapsules to obtain a mixture with a microcapsule content of about 20 to about 30 percent by weight, depositing the mixture containing microcapsules onto a carrier selected from the group consisting of a paper, paperboard, polymeric and porous substrate to provide a microcapsule containing substrate, drying the microcapsules containing substrate, and depositing a layer of an electron accepting compound on second substrate.

An advantage of the invention is that the images may be formed without the use of pigmented inks or dyes which may cause staining on clothing, skin or any other object which comes in contact with the colorless dye solution and which will not react with the colorless dye solution to develop the dye. Another advantage of the invention is that the components of the printing system are essentially dry until the microcapsules containing the dye or developing compound are ruptured, thereby reducing the amount of liquid components which may spill or otherwise volatilize before the system may be used by a consumer. Accordingly, the system is readily transportable and may be used in a variety of situations, particular with children, without worrying about having to clean the inks or dyes from objects contacted by the microcapsule containing substrate.

When the microcapsules are deposited on a substrate with a binder, substrate or ink pad may be discarded after an initial or single use unlike traditional ink pads which may be used multiple times. Since a moist pad is not required in order to use the printing system according to the present invention, there is less tendency for bacteria to accumulate on the microcapsule-containing substrate. By eliminating a

moist media which may promote the growth of bacteria, the transfer of bacteria from one individual to another is substantially reduced, particularly when contacting the microcapsule-containing substrate with the fingers of multiple individuals.

In yet another aspect, the invention provides a disposable ink pad and image producing system for producing images using an image containing object without visibly tinting the image containing object. The system comprises a paper or paperboard substrate having printed in a first region on the surface of the substrate, an essentially dry layer of microcapsules and binder wherein from about 50 to about 99 percent of the microcapsule weight is a colorless dye solution for depositing a colorless dye on the image containing object when the capsules are ruptured. A second coplanar region on the surface of the substrate is printed with a substantially dry dye developing layer for receiving the colorless dye from the image containing object to produce the image on the substrate in the second region upon contact with the colorless dye from the image containing object.

## BRIEF DESCRIPTION OF THE DRAWINGS

Other features and advantages of the invention will be described and understood by referring to the drawings in combination with the following description in which:

FIG. 1 is a cross-sectional view, not to scale, of the microcapsule containing substrate;

FIG. 2 is a cross-sectional view, not to scale, of a substrate containing a colorless dye or dye developing compound;

FIG. 3 is a perspective view of the substrate of FIG. 2 containing a colorless dye or dye developing compound;

FIG. 4 is a perspective view of a substrate containing both the microcapsule layer and the dye developing layer;

FIG. 5 is a perspective view of an image containing device;

FIG. 6 is a perspective view of another image containing device; and

FIG. 7 is a perspective view of a substrate containing a colorless dye first region and a printed dye developing compound in a second substrate region.

## DETAILED DESCRIPTION OF THE INVENTION

With reference to FIG. 1, there is provided an essentially dry disposable ink pad 10 comprising a substrate 12 having deposited thereon a layer 14 containing microcapsules 16. In addition to a coated paper or paperboard substrate 12, any porous media such as a foam pad which will absorb a mixture containing the microcapsules may be used as substrate 12. In the case of a paper or paperboard substrate, a binder 18 is typically used to adhere the microcapsules to the substrate 12. However, for other porous substrates, binders are not required.

The microcapsules 16 deposited on the substrate 12 contain a colorless solution 20 which is released from the ink pad 10 when the microcapsules are ruptured. The colorless solution 20 may be any dye compound or dye developer compound dispersed or dissolved in an oleaginous carrier fluid which optionally contains a minor amount, typically less than about 1 wt. %, of a fragrance imparting compound.

In order to provide sufficient colorless solution for transfer to a second substrate region containing a complementary compound for producing a visible image, it is preferred that the microcapsules 16 have an average effective spherical

diameter of from about 40 to about 80 microns. Since the microcapsules **16** are often elliptical in cross-sectional shape due to the method used to manufacture the microcapsules, the "effective spherical diameter" is the diameter of a sphere having substantially the same volume as the microcapsule. It is preferred that the amount of colorless solution **20** in each microcapsule **16** be from about 50 to about 99 percent by weight of the total weight of the microcapsule and solution.

The microcapsules **16** are designed to be deformable and not easily ruptured when contained in a carrier liquid so that the microcapsules can be deposited on a substrate **12** without rupturing or with only a minor amount of ruptured microcapsules **16**. Typically, less than about 2 percent by weight of the microcapsules may rupture during the deposition process used to deposit the microcapsules on a substrate.

In the case of a paper or paperboard substrate, the microcapsules **16** and binder **18** are preferably deposited on the first substrate region by a printing process rather than by coating the microcapsules and binder onto the substrate **12**. Printing of the microcapsule layer **14** provides more precise location of the microcapsule layer with respect to the portion of the substrate region to be used for the microcapsule layer. Printing methods which may be used to deposit the microcapsule layer **14** microcapsules **16** and binder **18** on a paper or paperboard substrate **12** may be selected from, but not limited to, flexo-graphic printing, silk screen printing and offset or gravure printing. The preferred printing method is a silk screen method wherein the silk screen has been prepared in ways well-known in the art so that a liquid microcapsule dispersion containing microcapsules, carrier liquid and/or binder may be deposited onto the desired area or areas of the substrate **12**.

During silk screen printing the microcapsule dispersion containing from about 20 to about 40 percent by weight microcapsules, preferably about 25 percent by weight microcapsules, and binder are placed on the surface of the silk screen or rubber plate opposite the substrate **12** and a squeegee is passed over the top surface of the screen or rubber plate in order to force the microcapsule dispersion and binder through the open portions of the screen or rubber plate and onto the substrate **12** to form the layer **14**. The mesh size of the silk screen or the percentage of line screen of the flexo-graphic plate is selected to allow a sufficient thickness of the layer containing microcapsules and binder to be deposited on the substrate. The preferred screen for silk screen printing is a 200 mesh screen with an opening size of approximately 125 microns and the weight of microcapsules and binder deposited using the preferred screen ranges from about 3 to about 6 pounds per 3000 square feet of substrate (about 4.7 to about 9.7 grams/m<sup>2</sup>), most preferably about 4 pounds per 3000 square feet (about 6.4 grams/m<sup>2</sup>) of substrate.

As was previously described, the microcapsules are of a construction which enables the microcapsules to be deformable while in a carrier liquid so that the shear forces incurred during the deposition process are insufficient to rupture the majority of the microcapsules. A preferred method for depositing microcapsules onto the surface of a substrate is disclosed in U.S. Pat. No. 3,578,482 to Whitaker et al. incorporated herein by reference as if fully set forth.

Subsequent to deposition, the layer **14** adheres to the substrate **12** by action of the binders and the substrate containing layer **14** is allowed to dry either by unassisted air drying or assisted heat drying. Upon drying, the layer **14** consists of a dried mixture of binder **18** and microcapsules

**16** which contain a colorless dye or dye developing compound in an oleaginous fluid **20**. After the layer **14** containing the binder **18** and microcapsules **16** has dried on the substrate **12** so that the microcapsules are effectively bound to the substrate, the microcapsule containing layer **14** is ready for use.

When the microcapsules **20** are deposited on a porous media such as a polymeric foam material such as polyurethane, open cell polyethylene and the like, a binder **18** is not required. The microcapsules **20** are simply deposited from a carrier liquid containing the microcapsules onto the porous media, and the media is then dried to remove the carrier liquid. Because the substrate is an open cell structure, a sufficient amount of microcapsules will be absorbed into or onto the substrate so that upon drying or evaporating the carrier liquid containing the microcapsules, an essentially dry microcapsule containing substrate is formed. By "essentially dry" means that the only significant liquid components present are those liquid components which are contained in the microcapsules and are released with the microcapsules are ruptured.

The colorless dye compound which is used for the methods and apparatus of the invention may be selected from one or more electron donating compounds such as vat dye intermediates which are often insoluble in water in their natural or oxidized state, but are colorless and soluble in water at a neutral or alkaline pH. Accordingly, the colorless dyes may be selected from, but not limited to, lactones, dilactones, derivatives of bis-(p-dialkylaminoaryl)methane, zanthenes, indolyls, auramines, fluorans, bisfluorans. Specific colorless dyes include, indigo, inanthrene blue, benzoyl leuco methylene blue, 3,3-bis(1'-n-octyl-2'-methyl-indol-3'-yl)phthalide, crystal violet lactone, 2-(N-benzyl-N-noctyl) amino-6-diethylaminofluoran and 6'-(diethylamino)-3'-methyl-2'-(phenylamino)spiro(isobenzofuran-1(3H),9'-(9H) xanthen)-3-one.

The colorless dye is preferably dissolved in an oleaginous material. Typically, the colorless dye solution will contain from about 10 to about 20 percent by weight of colorless dye and from about 80 to about 90 percent by weight of oleaginous material. The oleaginous material may be selected from a citrus oil such as lemon oil, orange oil, grapefruit oil or lime oil, a water insoluble fatty acid, an aliphatic ester and similar oleaginous materials.

When a binder **18** is used to bind the microcapsules **16** to the substrate **12**, the binder may be selected from gum arabic, methyl cellulose, polyvinyl alcohol, starch, polyacrylic acid, carboxymethyl cellulose, ethylcellulose, cellulose acetate, polyvinyl acetate, polyvinylpyrrolidone, polyacrylamide, shellac, natural gums, hydroxypropyl cellulose and other compounds having similar properties. Preferred binders include methyl cellulose and hydroxypropyl cellulose.

Another important component of the printing system according to the invention is a dye developing compound. The dye developing may be provided as a liquid component of the microcapsules as described above or may be provided in an essentially dry layer **32** which is deposited on a second substrate region or in a second substrate region on the first substrate. When contacted with the colorless dye solution, the dye developing compound in layer **32** reacts with the dye solution to oxidize the dye and convert the dye to the colored or tinted form.

Preferred dye developing compounds are compounds which are electron-accepting substances and may be selected from, but not limited to, acidic clays such as

montmorillonites, kaolins, talc, bentonites, and attapulgites; phenolic resins; metal oxides; metal chlorides; derivatives of aromatic carboxylic acids and their metal salts, aliphatic dicarboxylic acids and novolac phenolic resins. Examples of one or more dye developing compounds which may be used include, but are not limited to, aluminum silicate, calcium citrate, 4-tert-butylphenol, 4-phenylphenol, 4-hydroxydiphenyloxide,  $\alpha$ -naphthol, 4-hydroxybenzoic acid methyl ester,  $\beta$ -naphthol, 4-hydroxyacetophenone, 2,2'-dihydroxydiphenyl, 4,4'-isopropylidenediphenol, 4,4'-isopropylidene-bis-(2-methylphenol), 4,4'-bis(hydroxyphenyl) valeric acid, hydroquinone, pyrogallol, chlorogluconol, p-, m-, o-hydroxybenzoic acid, gallic acid, 1-hydroxy-2-naphthoic acid, boric acid, tartaric acid, oxalic acid, maleic acid, citraconic acid and succinic acid. A particularly preferred dye developing compound is an alkylphenol novolac resin dispersion which is commercially available from Schenectady International, Inc. of Schenectady, N.Y. under the trade name HRJ-4023.

As with the microcapsule layer 14, a dye developing layer 32 is preferably deposited on the substrate 30 by any of the beforementioned printing methods with a conventional flexo-graphic printing method being the most preferred. Binders such as those for use with the microcapsule layer 14 may also be used to adhere the dye developing layer 32 to the substrate 30. However, when the dye developing compound is an alkylphenol novolac resin, no additional binders are required as the resin itself acts as a binder. The amount of dye developing compound deposited on the substrate preferably ranges from about 1 pound per 3000 square feet (1.6 grams/m<sup>2</sup>) to about 3 pounds per square feet (4.7 grams/m<sup>2</sup>), preferably about 2 pounds per 3000 square feet (3.2 grams/m<sup>2</sup>).

The dye developing compound may be deposited on the same paper or paperboard substrate 12 in a second substrate region with respect to a first region containing the microcapsule layer or on a separate paper or paperboard substrate 30. When deposited on the same substrate as the microcapsule layer, it is preferred to deposit the dye developing layer 32 in a spatially separate, coplanar location on the same surface of the substrate 12 as the microcapsule layer 14. FIG. 4 illustrates a substrate 40 having both the microcapsule layer 42 containing colorless dye solution and the dye developing layer 44 of a substantially dry dye developing compound. Once deposited on the substrate 30 or 40, the dye developing layer 32 is dried by air or heat so that the layer is substantially dry to the touch.

In addition to porous media, paper and paperboard substrates, the layers 14 and 32 may be deposited on other materials such as, but not limited to, coated paper, wood, plastic or metal.

In order to use the printing system according to the invention, a plurality of microcapsules 16 are broken by pressure from an image containing object and a portion of the colorless solution 20 is transferred to the surface of the image containing object. Next, at least a portion of the colorless solution 20 which was transferred to the image containing object is transferred to the second substrate region containing either the complementary dye or dye developing compound 32, depending on whether the microcapsules contain a dye or dye developing compound, by contacting the second substrate region with the image containing object. Contact between the colorless dye solution 20 and the dye developing compound causes a reaction between the colorless dye solution 20 and the color developing compound so that an oxidized form of the dye, which is highly colored, is provided.

Suitable image containing objects 46 and 60 are illustrated in FIGS. 5 and 6 respectively. The image containing object 46 or 60 may contain a rigid base 48 or 62 and a handle 50 or 64 fixedly attached to one surface 52 or 66 of the base 48 or 62 respectively. An opposing surface 54 or 68 of the image containing object 46 or 60 contains an image 56 or 70 which has a surface 58 or 72 respectively, substantially parallel to and offset from the surface 54 or 68 of the object 46 or 60. It is preferred that only surface 58 or 72 retain the portion of colorless dye 20 as a result of contacting the image containing object 46 or 60 with the substrate containing the microcapsules 16. The surface 58 or 72 should not be so absorbent however, that it inhibits the subsequent transfer of a portion of the liquid obtained from the microcapsules to a second substrate region containing the complementary dye or dye developing compound 32.

The image portion 56 or 70 of the image containing object 46 or 60 may be made from an elastomeric material such as natural or synthetic rubber which may be attached by a suitable adhesive or any other attachment method known to those of skill in the art to a plastic or wooden rigid base 48 or 62. Other image containing objects may also be used including, but not limited to, metal dyes, fingers and other useful or ornamental surfaces having sufficient relief for the contact and transfer of colorless dye from the microcapsules to the second substrate region which contains a compound which reacts with the transferred liquid to produce a visible image.

In another embodiment, there is provided an image producing system comprising a first substrate region comprising an essentially dry layer of fluid filled microcapsules and binder. The microcapsules in the first substrate region preferably have an average spherical diameter of from about 40 to about 80 microns and contain a fluid selected from the group consisting of colorless dye solutions, preferably a colorless vat dye solution as described herein and dye developing solutions, preferably an alkylphenol novolac resin solution. There is also provided a second substrate region having printed thereon a substantially dry compound which compound is reactive with the fluid from the microcapsules and wherein the compound is printed on the second substrate region in the shape of text or a design. An important aspect of the invention is that the printed compound is substantially imperceptible prior to reaction with the microcapsule fluid and the printed compound becomes visible subsequent to reaction with the microcapsule fluid. One use for the image developing system is as a game piece or game board wherein contact between the fluid from the microcapsules and the area of the second substrate region containing the image to be developed produces a visibly correct or incorrect answer to a question.

FIG. 7 illustrates various features of the image producing system 78 according to the invention. In this embodiment, there is provided a substrate 80 having a first substrate region 82 comprising an essentially dry layer 84 of fluid filled microcapsules and binder and a second substrate region 86 having printed thereon a substantially dry compound in the shape of text or a design. The second substrate region may contain a single design or text in a single location, or may, as illustrated in FIG. 7, the second region may contain a plurality of sections each containing text or a design. The compounds 88, 90 and 92 printed in sections 94, 96 and 98 respectfully of the second substrate region are shown in outline form to represent designs or text which are substantially imperceptible before contact with the fluid from the microcapsules. The compound 100 in section 102 of the second substrate region is in solid form to represent

the compound after reaction with the fluid from the micro-capsules. After reaction between the microcapsule fluid and the compound in section 102 of the second region 86, the image becomes visible whereas the images in sections 94, 96 and 98 remain substantially imperceptible in the absence of reaction between the microcapsule fluid and the compound in those sections.

In order to use the image producing system illustrated in FIG. 7, an object such as a finger or absorbent media having sufficient relief to provide an image thereof is pressed or rubbed on the microcapsule layer 84 with a pressure sufficient to break at least a portion of the microcapsules and release fluid to the object. The object may then be rubbed over or pressed on the second substrate region 86 in a selected area so that sufficient fluid from the object may be transferred from the object in order to react with the printed compound so that the image may change from substantially imperceptible to visible as shown in section 102 by design 100.

In another aspect, the invention provides a method for making an essentially dry printing system. The method comprises milling an aqueous gelatin mixture containing water, a solution containing about 10 to about 20 percent by weight of a vat dye or dye developing compound and about 80 to about 90 percent by weight of an oleaginous material to an oil droplet size of about 40 to about 80 microns. The milled dye droplets in the aqueous gelatin mixture are then dispersed in an aqueous gum arabic solution while mixing the dispersion at a speed sufficient to maintain the particle size. During mixing, the dispersed mixture is cooled to a temperature in the range of from about 5 to about 15° C., preferably about 10° C. When the desired temperature is obtained, a crosslinking agent is added to the dispersed mixture to form the microcapsules. The cooled solution is then maintained under agitation for from about 10 to about 20 hours at a pH of about 4.5. At the end of the holding period, water is removed from the dispersed mixture containing microcapsules, preferably by filtration, to obtain a mixture with a microcapsule content of about 20 to about 30 percent by weight. The microcapsule containing mixture is then deposited, preferably by a printing process, with a binder in a first substrate region on a surface of a paper or paperboard substrate to provide a microcapsule and binder layer and the microcapsule and binder layer is dried. A layer of an electron accepting compound and binder is printed in a second substrate region on the surface of a substrate, preferably the same surface of the same substrate in a spatially separate, coplanar location with respect to the microcapsule and binder layer.

The microcapsule layer may contain other ingredients in addition to the colorless dye. Accordingly, a fragrance compound may be included with the colorless dye compound or dye developer compound to give the image a distinctive fragrance. Fragrances which may be used include the natural citrus oils such as lemon, grapefruit, lime and orange oils, spearmint as well as synthetic fragrances such as strawberry, watermelon and chocolate. The amount of fragrance in the microcapsules is typically less than about 1 wt. % of the microcapsule fluid.

The following example illustrates a process for preparing a microcapsule layer 14 containing colorless dye solution according to the invention.

#### EXAMPLE 1

A mixture of 90 mL of an 11 wt. % aqueous gelatin solution, 120 mL of COPIKEM 4 (a black colorless dye

solution containing an oleaginous material available from Hilton Davis Co. of Cincinnati, Ohio) and 100 milliliters of water were milled in a WARING blender on a medium speed at a temperature of about 35° C. and a pH in the range of 4.75 to 5.0 for a period of time sufficient to obtain emulsified droplets having an average effective spherical diameter of about 40 to about 80 microns. The emulsion was then added to a 1000 mL beaker containing 90 mL of an 11 wt. % gum arabic solution, and 300 mL of dilution water while agitating the mixture at a speed sufficient to maintain the particle size of 40 to 80 microns. The resulting system was cooled slowly from 35° C. to 26° C. over a period of 4 hours. At 26° C. the pH of the system was lowered to 4.5 using acetic acid. After adjusting the pH, the 1000 mL beaker containing the liquid was placed in an ice bath to quickly cool the system to 10° C. At this point, 5 mL of glutaraldehyde were added to assist in solidification of the microcapsule walls. At this point the liquid contained about 20 wt. % microcapsules dispersed in water. The microcapsules were concentrated to about 25 wt. % by filtration and 1 wt. % each of methylcellulose and KLUCEL resins (commercially available from Aqualon of Wilmington, Del.) were added to the dispersed microcapsules. The mixture was then printed onto a paperboard substrate by a silk screen printing process using a 200 mesh screen to provide 4 pounds per 3000 square feet (6.4 grams/m<sup>2</sup>) of the microcapsule layer. The printing process used was generally in accordance with the procedure disclosed in U.S. Pat. No. 3,758,482 to Whitaker et al. incorporated herein by reference as if fully set forth. The printed product was allowed to dry completely.

The substrate containing the dye developing compound was prepared according to the following example.

#### EXAMPLE 2

An aqueous emulsion of an alkylphenol novolac resin dispersion containing 55 weight percent solids (trade name HRJ-4023 commercially available from Schenectady International, Inc. of Schenectady, N.Y.) was deposited by a conventional flexo-graphic printing process on a paperboard substrate. The coating thickness was about 2 pounds per 3000 square feet (3.2 grams/m<sup>2</sup>). The dye developing layer was allowed to dry completely before use.

Slight pressure was used to contact and rub the micro-capsule containing layer with a finger to break a portion of the microcapsules and obtain a portion of the colorless dye on the finger. The finger was then pressed to the portion of a substrate containing the dye developing layer. A black image of the fingerprint was obtained on the dye developing coating with no transfer of color to the finger.

In yet another embodiment of the printing system according to the invention, the microcapsule layer illustrated in FIG. 1 contains the dye developing compound dissolved in a suitable hydrophobic solvent such as xylene or toluene, and the layer illustrated in FIGS. 2 and 3 contains a substantially dry coating of a colorless dye compound. In all other aspects, the methods and uses of the foregoing printing system of the invention is substantially the same as the system wherein the microcapsules contain the colorless dye.

Having described and illustrated preferred embodiments of the invention, it will be recognized that the substrate and/or either of the layers on the substrate may contain other ingredients which do not interfere with the performance of the colorless dye or dye developing compound. For example, the substrate may be precoated with a pigment or other coating to indicate the position of the dye developing layer and/or the microcapsule layer. Either or both layers

may contain fragrances to enhance the aesthetics of the coated substrates. One or both substrates may contain printed indicia or figures for functional or ornamental purposes. Numerous other modifications, substitutions and additions may be made to the invention within the spirit and scope of the appended claims by those of ordinary skill.

What is claimed is:

1. An essentially dry ink pad containing an essentially colorless composition for use with a complementary essentially colorless compound to develop a visible image which comprises a porous substrate impregnated with substantially dry microcapsules, said microcapsules containing an essentially colorless dye compound, an oleaginous fluid and a fragrance.

2. The essentially dry ink pad of claim 1 wherein the microcapsules have a spherical diameter within the range of from about 40 to about 80 microns.

3. The essentially dry ink pad of claim 1 wherein the dye compound comprises an electron donating dye.

4. The essentially dry ink pad of claim 3 wherein the dye compound comprises a vat dye.

5. The essentially dry ink pad of claim 1 wherein the microcapsules contain from about 10 to about 20 weight percent colorless dye and from about 80 to about 90 weight percent citrus oil.

6. An essentially dry ink pad containing an essentially colorless dye developer compound for use with a complementary essentially colorless dye compound which comprises a porous substrate impregnated with substantially dry microcapsules, said microcapsules containing an essentially colorless dye developer compound, oleaginous fluid and a fragrance.

7. The essentially dry ink pad of claim 6 wherein the microcapsules have a spherical diameter within the range of from about 40 to about 80 microns.

8. The essentially dry ink pad of claim 6 wherein the dye developer compound comprises an electron accepting compound.

9. The essentially dry ink pad of claim 8 wherein the dye developer compound comprises a phenolic derivative.

10. The essentially dry ink pad of claim 8 wherein the microcapsules contain from about 10 to about 20 weight percent dye developer compound and from about 80 to about 90 weight percent citrus oil.

11. A method for making an essentially dry printing system, the method comprising:

millling an aqueous gelatin mixture containing water, a solution containing from about 10 to about 20 percent by weight of an electron donating dye compound and from about 80 to about 90 percent by weight of an oleaginous material to a particle size of about 40 to about 80 microns;

dispersing the milled aqueous gelatin mixture in an aqueous gum arabic solution while mixing the dispersion at a speed sufficient to maintain the particle size;

cooling the dispersed mixture to a temperature in the range of from about 5 to about 15° C.;

adding a cross-linking agent to the cooled mixture to form microcapsules;

maintaining the cooled mixture under agitation for from about 10 to about 20 hours at a pH of about 4.5; removing water from the mixture containing microcapsules to obtain a mixture with a microcapsule content of about 20 to about 30 percent by weight;

impregnating a porous substrate with the mixture containing microcapsules; drying the microcapsules containing substrate; and depositing a layer of an electron accepting compound on second substrate.

12. The method of claim 11 wherein the dye compound comprises a vat dye.

13. The method of claim 11 wherein the electron accepting compound comprises an alkylphenol novolac resin.

14. The method of claim 11 wherein the microcapsules contain from about 10 to about 20 weight percent colorless dye compound and from about 80 to about 90 weight percent of a citrus oil.

15. The method of claim 11 wherein the cross-linking agent is glutaraldehyde.

16. A method for making an essentially dry printing system, the method comprising:

millling an aqueous gelatin mixture containing water, a solution containing from about 10 to about 20 percent by weight of an electron accepting compound and from about 80 to about 90 percent by weight of an oleaginous material to a particle size of about 40 to about 80 microns;

dispersing the milled aqueous gelatin mixture in an aqueous gum arabic solution while mixing the dispersion at a speed sufficient to maintain the particle size;

cooling the dispersed mixture to a temperature in the range of from about 5 to about 15° C.;

adding a cross-lining agent to the cooled mixture to form microcapsules;

maintaining the cooled mixture under agitation for from about 10 to about 20 hours at a pH of about 4.5;

removing water from the mixture containing microcapsules to obtain a mixture with a microcapsule content of about 20 to about 30 percent by weight;

impregnating a porous substrate with the mixture containing microcapsules;

drying the microcapsules containing substrate; and depositing a layer of an electron donating dye compound onto a second substrate.

17. The method of claim 16 wherein the dye compound comprises a vat dye.

18. The method of claim 16 wherein the electron accepting compound comprises an alkylphenol novolac resin.

19. The method of claim 16 wherein the microcapsules contain from about 10 to about 20 weight percent electron accepting compound and from about 80 to about 90 weight percent of a citrus oil.

20. The method of claim 16 wherein the cross-linking agent is glutaraldehyde.

UNITED STATES PATENT AND TRADEMARK OFFICE  
**CERTIFICATE OF CORRECTION**

PATENT NO. : 5,942,464

DATED : August 24, 1999

INVENTOR(S) : Vaughn et al

It is certified that error appears in the above-identified patent and that said Letters Patent is hereby corrected as shown below:

In Column 1, line 62, before "substrate" insert --the--.

In Column 5, line 44, after "layer 44" insert --made--.

In Column 5, line 46, after "layer 32" insert --or 44--.

In Column 5, line 67, change "provided" to --produced--.

In the claims:

Col. 10, Claim 11, line 11, before "second" insert --a--.

Signed and Sealed this

Twenty-third Day of May, 2000

Attest:



Q. TODD DICKINSON

Attesting Officer

Director of Patents and Trademarks